

1

3,382,055

## POLYALKYLETHYLENEOXIDE POUR POINT DEPRESSANT ADDITIVE

Norman Jacobson and Herbert G. Burkard, Roselle, N.J., assignors to Esso Research and Engineering Company, a corporation of Delaware  
No Drawing. Filed Feb. 24, 1965, Ser. No. 435,031  
2 Claims. (Cl. 44—62)

### ABSTRACT OF THE DISCLOSURE

Polymers of 1,2-epoxy alkanes having 10 to 18 carbon atoms, wherein the molecular weight is in the range of 1,000 to 1,000,000 are pour depressants for middle distillates and light lube oil stocks.

The present invention is broadly concerned with an additive for improving the quality of middle distillates and light lube oil stocks. The present invention relates to improving the flow at low temperatures and the pour characteristics of middle distillates and lube oil stocks. More particularly, the present invention relates to the manufacture of improved pour depressants for use with these middle distillates, in particular, heating oils and diesel fuels, kerosene, aviation turbojet fuels, and other fuels and lubricating oils that are subject to low temperatures. The additives of the present invention are polymers derived from 1,2-epoxy alkanes.

With the increase in the use of hydrocarbon fuels of all kinds, a serious problem has arisen in areas frequently subjected to low temperatures with respect to the cold characteristics of these fuels. Particularly, serious problems have been encountered with heating oils, diesel oils and jet fuels that have too high a pour point, resulting either in distributional or operating difficulties or both. For example, the distribution of heating oil by pumping or siphoning is rendered difficult or impossible at temperatures around or below the pour point of the oil. Furthermore, the flow of the oil at such low temperatures through the filters cannot be maintained, leading to the operating failure of the equipment.

Particularly the low temperature properties of petroleum distillate fuels boiling in the range between about 250° and about 750° F. have attracted increased attention in recent years because of the growth of markets of such fuels in subarctic areas and also because of the development of turbojet aircraft capable of operating at altitudes where temperatures of —50° F. or lower may be encountered.

Thus it is one object of the present invention to provide heating oils, diesel fuel oils, kerosenes and jet fuels having low pour points. Aviation turbojet fuels in which the polymers of the present invention may be used normally boil between about 250° and about 550° F. and are used in both military and civilian aircraft. Such fuels are more fully defined by U.S. Military Specifications MIL-F-5624C, MIL-F-25554A, MIL-F-25558A, and amendments thereto. Kerosenes and heating oils will normally have boiling ranges between about 300° and about 750° F. and are more fully described in ASTM Specification D-396-48T and supplements thereto, where they are referred to as No. 1 and No. 2 fuel oils. Diesel fuels in which the polymers may be employed are described in detail in ASTM Specification D-975-35T and later versions of the same specification.

The light lube oils with which the present invention is concerned are petroleum neutral oils having viscosities in the range from 100 to 300 Saybolt seconds at 100° F.

The polymeric pour depressants may, in accordance

2

with the invention, be employed in conjunction with a variety of other additives commonly used in fuels such as those set forth above. Typical of such additives are rust inhibitors, anti-oxidants, dispersants, dyes, dye stabilizers, haze inhibitors, antistatic agents and the like. It will frequently be found convenient to prepare additive concentrates for use in the various types of fuels and thus add all of the additives simultaneously.

In essence, the additives of the present invention consist essentially of polymers obtained from 1,2-epoxy alkanes. The molecular weights of the polymers are in the range from about 1,000 to 1,000,000, preferably in the range from about 1,000 to 3,000 for heating oils and from 50,000 to 150,000 for lube oils. The molecular weights are determined by K. Rast's method (Ber. 55, 1051, 3727 (1922)). The polymers are derived from 1,2-epoxy alkanes and have a structural formula as follows:



wherein  $n$  is 8 to 16, preferably 10 to 14 and wherein  $x$  is 6 to 600, preferably 10 to 20. The epoxy compound



is prepared by starting with a monoolefin containing from about 10 to 18 carbon atoms in the molecule, preferably a  $\text{C}_{14}$  olefin. It is essential that the double bond be between the thirteenth and fourteenth carbon atoms.

The polymers as described in the present invention are used in the base oil in a concentration in the range from about .001 to 0.2% by weight, preferably in a concentration in the range from about .005 to 0.1% by weight.

The present invention may be more fully understood by the following examples illustrating the same.

### EXAMPLE 1

A poly-1,2-epoxy tetradecane was prepared as follows: 200 parts of 1-tetradecene and 200 ml. of methylene chloride were added to a 5 liter flask equipped with a stirrer, thermometer and condenser. m-Chloroperbenzoic acid (205 parts) (85% pure) was dissolved in 1800 parts methylene chloride and gradually added to the olefin solution at such a rate that the reaction temperature did not rise above 40° C. After completion of the addition, the reaction solution was stirred overnight (16 hrs.). The reaction solution gave a negative test with starch-iodide paper and was filtered to remove the m-chloroperbenzoic acid. The reaction solution was washed with 5% sodium bicarbonate solution and then with water. The methylene chloride was nitrogen stripped overnight at room temperature and the residual liquid distilled. The portion boiling at 122° to 124° C./3.0 mm. was collected. The product 1,2-epoxy tetradecane (94.1 parts) was obtained as a colorless liquid.

The monomer, 1,2-epoxy tetradecane, is then polymerized utilizing a catalyst such as boron trifluoride-etherate to obtain low molecular weight product in the range from about 2,000 to 10,000. A diluent may or may not be used and the catalyst may be suspended or dissolved in the diluent. The reaction proceeds at a temperature in the range from about —70° to 50° C., preferably at about 8° C. for a period of about 1 to 4 hours, such as about 2 hours.

High molecular weight products in the range from about 10,000 to 100,000 are obtained by the use of a coordinated anionic catalyst such as diethyl zinc-water or triethyl aluminum-water. An inert diluent such as pentane,

hexane, benzene, xylene, etc., may be used. This reaction can be conveniently run at a temperature in the range from about 0° to 150° C. (depending on the diluent used); preferably at about 70° C.

Other polymers were prepared using the following 5 epoxy alkanes: C<sub>12</sub>, C<sub>11</sub>-C<sub>15</sub> and C<sub>16</sub>-C<sub>18</sub> using the technique described.

#### EXAMPLE 2

Approximately 16 parts monomer (1,2 - epoxy tetradecane) were polymerized in 12.5 parts pentane by the gradual addition of 1 ml. BF<sub>3</sub>·etherate suspended in 3.2 parts pentane. The reaction was run at 8° C. for a period of 1 hour and then gradually allowed to warm to room temperature. Additional pentane (30 parts) was added 10 to the reaction mixture and the organic phase was washed several times with water. It was next dried over anhydrous sodium sulfate and filtered. The pentane was removed by nitrogen stripping and the residue placed in a vacuum oven at 60° C./125 mm. Hg. The crude residue 20 was dialyzed to obtain a pure product.

#### EXAMPLE 3

Approximately 16 parts monomer (1,2 - epoxy tetradecane) were polymerized without a diluent by the gradual addition of 1 ml. BF<sub>3</sub>·etherate in 3.2 parts pentane. The reaction was run at 8° C. for a period of 2 hours. Pentane (75 parts) was added and the product was obtained according to the procedure described in Example 2. 25

#### EXAMPLE 4

Following the procedure described in Example 3, a mixture of 8.3 parts 1,2 - epoxy dodecane and 8.3 parts 35 1,2 - epoxy tetradecane were polymerized by the gradual addition of 1 ml. BF<sub>3</sub>·etherate dissolved in 3.6 parts ethyl ether. The reaction was run at 8° C. for 2 hours. A crude yield of 16.3 parts residue was obtained.

#### EXAMPLE 5

Following the procedure described in Example 3, approximately 16 parts of a commercially available mixture of terminal epoxide composition 1,2 - epoxy undecane, 45 1,2 - epoxy dodecane and 1,2 - epoxy tridecane were polymerized yielding 8.1 parts of a crude polymeric product.

#### EXAMPLE 6

Following the procedure described in Example 3, approximately 17 parts of a mixture of 1,2 - epoxy hexadecane (40%) and 1,2 - epoxy octadecane were polymerized at 13° C. by the gradual addition of 1 ml. 50 55 BF<sub>3</sub>·etherate suspended in 3.2 parts pentane giving 9.6 parts of a crude product which was a semi-solid.

#### EXAMPLE 7

A liquid mixture of 44 parts benzene, 12.4 parts 1,2- 60 epoxy dodecane and 0.05 part water was prepared in a screw cap bottle equipped with a Teflon coated magnetic stirring bar. While the mixture was stirred, 0.74 part diethyl zinc was added (as a 3 m. solution in benzene). The operations were conducted in a nitrogen dry box. The bottle was capped and transferred to a constant temperature bath at 50° C. for 24 hours. The reaction mixture was dissolved in 2 liters of benzene, washed first with 1 liter of water containing 10 ml. 12 N hydrochloric acid, then with an additional liter of water. The solution was dried over anhydrous sodium sulfate and filtered. The benzene was removed by nitrogen stripping at 75° to 85° C. The resulting polymer was dried in a vacuum oven and the product yield was 10.9 parts.

#### EXAMPLE 8

Following the procedure of Example 7, a mixture of 44 parts of benzene, 12.4 parts 1,2 - epoxy dodecane and 0.69 part triethyl aluminum was reacted at 70° C. for 24 hours. The product recovery technique of Example 7 was used to give 11.1 parts of polymer having an intrinsic viscosity of 0.83 in toluene at 20° C.

#### EXAMPLE 9

Following the procedure of Example 7, a mixture of 44 parts of benzene, 12.4 parts 1,2 - epoxy dodecane, 0.05 part water and 2.34 parts of trioctyl aluminum was reacted at 70° C. for 24 hours. The product recovery technique of Example 7 gave a yield of 11.2 parts polymer which had an intrinsic viscosity of 0.21 in toluene at 20° C.

#### EXAMPLE 10

Following the procedure of Example 7, a mixture of 44 parts of benzene, 12.4 parts of 1,2 - epoxy dodecane, 0.05 part water and 1.07 parts triisobutyl aluminum was reacted at 70° C. for 24 hours. The product recovery technique of Example 7 gave a yield of 11.4 parts polymer having an intrinsic viscosity of 0.91 in toluene at 20° C.

#### EXAMPLE 11

Following the procedure of Example 7, a mixture of approximately 12.5 parts C<sub>11</sub>-C<sub>15</sub> olefin oxide (a mixture of mainly terminal epoxides C<sub>n</sub>H<sub>2n</sub>O where n=11 to 15), 44 parts benzene, 0.05 part water and 1.07 parts triisobutyl aluminum was reacted at 70° C. for 24 hours. In attempting to dissolve the reaction mixture into benzene, a good portion of the product was found to be insoluble. The benzene suspension was filtered and 7.05 parts of polymer (insoluble in oil and benzene) was obtained. The filtrate was treated according to the product recovery technique described in Example 7 and 3.55 parts (oil and benzene soluble) polymer were obtained.

The polymers of Examples 2 to 11 were tested as pour point depressants in a fuel oil and in a light lube oil. The results are shown in Tables I and II.

Table I.—Pour point data on polymers in fuel oil

| Fuel oil 1: Oil+0.1 wt. percent polymer of Example— | Pour point (°F.) |
|-----------------------------------------------------|------------------|
| 2                                                   | -55              |
| 3                                                   | -60              |
| 4                                                   | -55              |
| 5                                                   | -15              |
| 6                                                   | -45              |
| 7                                                   | -20              |
| 8                                                   | -15              |
| 9                                                   | -20              |
| 10                                                  | -20              |
| 11                                                  | -20              |

<sup>1</sup> Fuel oil was approximately 50/50 vol. percent straight run and cracked stocks from a mixture of Venezuela and Gulf Coast crudes. The following are typical specifications:  
Cloud point °F. +4  
Pour point °F. -5  
Aniline point °F. 132  
Viscosity SUS/100° F. 34.2  
API gravity g./60° F. 33.0  
Density g./60° F. 0.860

Table II.—Pour point data on polymers in Mineral oil  
Pour point (°F.)

| Mineral oil 1<br>Oil+0.1 wt. percent polymer of Example— | 15  |
|----------------------------------------------------------|-----|
| 7                                                        | -5  |
| 8                                                        | 0   |
| 9                                                        | -5  |
| 10                                                       | -10 |
| 11                                                       | -5  |

<sup>1</sup> A solvent refined neutral mineral lubricating oil having 75 a viscosity of 169.3 SUS at 100° F.

What is claimed is:

1. A distillate fuel oil boiling between about 250° F. and 750° F. improved in pour point by the incorporation therein of a pour depressing effective amount within the range from about .005 to .2% by weight of an oil soluble polymer having a structural formula as follows:



wherein  $n$  is 8 to 16 and  $x$  is from 6 to 600.

2. A composition as defined by claim 1, wherein  $n$  is 10 to 14,  $x$  is 10 to 20, and said polymer has a Rast molecular weight of about 1,000 to 3,000.

References Cited

UNITED STATES PATENTS

|           |         |                      |         |
|-----------|---------|----------------------|---------|
| 2,457,328 | 12/1948 | Swern et al. _____   | 252—52A |
| 2,379,728 | 7/1945  | Lieber et al. _____  | 44—62 X |
| 2,544,375 | 3/1951  | Butler _____         | 252—52  |
| 2,786,745 | 3/1957  | Stayner et al. _____ | 44—62 X |
| 3,030,316 | 4/1962  | Bailey _____         | 260—615 |

10 DANIEL E. WYMAN, *Primary Examiner.*

W. J. SHINE, *Assistant Examiner.*

UNITED STATES PATENT OFFICE  
CERTIFICATE OF CORRECTION

Patent No. 3,382,055

May 7, 1968

Norman Jacobson et al.

It is certified that error appears in the above identified patent and that said Letters Patent are hereby corrected as shown below:

Column 5, lines 7 and 8, the formula should appear as shown below:



Signed and sealed this 16th day of December 1969.

(SEAL)

Attest:

Edward M. Fletcher, Jr.

Attesting Officer

WILLIAM E. SCHUYLER, JR.

Commissioner of Patents